

## UNITED STATES PATENT OFFICE

WILLIAM H. MASON, OF LAUREL, MISSISSIPPI, ASSIGNOR TO MASONITE CORPORATION, OF LAUREL, MISSISSIPPI, A CORPORATION OF DELAWARE

## PROCESS OF MAKING INTEGRAL INSULATING BOARD WITH HARD WELDED SURFACES

No Drawing. Original application filed March 1, 1926, Serial No. 91,447. Divided and this application filed March 16, 1928. Serial No. 262,336.

My invention relates to the process of making an integral insulating board having a porous interior and hard welded surfaces. The present application is a division of my prior copending application Serial No. 91,447 filed March 1st, 1926, issued as Patent Number 1,663,506 of March 20, 1928.

Ligno-cellulose materials of various kinds, such as wood and the like can be used for making my improved product, but for convenience I refer herein especially to wood as a source of material.

The principal object of the invention is the production from natural wood, such as waste pieces from saw mills, of an integral board product, the interior or backing portion of which is of relatively high porosity and is a good insulator, and the surface portion or portions whereof are hard, dense, stiff and strong, both the interior and surface portions being produced from an integral body of fiber.

Other objects will appear in the following description of my product and the process of its making.

The raw material, such as wood in small pieces or chips, is first converted into fiber. The fiber is preferably prepared by explosion from a gun through a constricted outlet or outlets under high pressure, preferably steam pressure, of about 250-1000# per square inch, but the wood may be ground or fibrated in other ways, so long as the lignins or a material part thereof are retained, and the fibers are not unduly chopped or shortened. Chemically digested fibers from which the lignins have been removed are not adapted for the purposes of my invention. To secure the best embodiment of my invention the fiber should contain all or practically all of the original wood or woody material disintegrated into fibrous state. Without commitment to a particular theory I believe that the lignins, which are plastic under conditions of heat, moisture and pressure herein-after described, serve for producing a welding or coalescing of the cellulose fibers in the surface portion of my product solidly together, so that said surface portion for practical purposes consists practically of wood

remade in modified form, with the fibers rearranged without grain or order, and of increased density and hardness.

After being fibrated, as, for example, by explosion from a gun, refinement as by beating and the like need not be resorted to and if there is any further refinement same is not extensive. The exploded fiber direct from the gun can be made use of, if desired, for the purposes of the present invention, without refinement.

The fiber is preferably formed into a felted sheet from a water bath, which may contain materials for making the product more waterproof or fire resistant or both.

Some of the excess water may be eliminated as by passing through squeezing rolls. This is, however, largely a matter of convenience, as the squeezing or wringing out of water, which takes place to some extent in any case in connection with the drying, can all be performed in such connection.

In the fibration and formation in water into felted sheets or the like form, the natural substantially parallel arrangement of the fibers existing in the wood is lost and the fibers become criss-crossed in various directions, so that the resulting product is grainless and of substantially like strength and stiffness in all surface directions.

The sheet or other form of fibrated material is subjected in moist form to heat and pressure. When in sheet form, the fiber sheet is cut into lengths as desired, and the sections introduced into a heated press, as, for example, for the production of products which are hard surfaced on both sides, between upper and lower steam heated press platens.

When the moist fiber sheet is compressed between the hot press platens, the pressure throughout the entire fibrous mass is substantially uniform, but the heat penetrates relatively slowly from the surfaces of the hot press platens toward the interior or center of the fibrous mass in the press. The welding of the cellulose fibers by their lignins appears to take place progressively inwardly beginning from the hot platen surfaces and extending gradually inward as the heat pen-

etrates into the interior and toward the center of the mass of fiber.

If the compression is sufficiently high and is maintained for a sufficiently long time to permit the heat to penetrate throughout the mass of fiber, this welding action will be substantially complete throughout the entire thickness of the fibrous mass as is set forth and claimed in my copending application Serial No. 57,252, filed September 18, 1925, issued as Patent Number 1,663,505 of March 20, 1928.

After an interval of time has elapsed, however, such that heat penetration and welding extends only part way in, and the welding is not yet complete all the way through, the mass of fiber between the press platens would be found to consist of hard, dense, welded surface portions separated by an interior felted portion, which, while being subjected to the same pressure as the surface portions, has not yet become welded because of the heat not yet having penetrated sufficiently to produce welding in such region. When the fibrous body is in this condition the application of heat is stopped or heat is reduced to a point below the temperature required for welding or coalescing the fibers together, as for example by cutting off the supply of steam to the press platens or by introducing water therein. The inwardly progressive coalescing or welding of the fibers is interrupted as mere application of pressure is insufficient to produce the effect of coalescing or welding of the fibers in the absence of sufficient heat. Upon opening the press at this stage, the central unwelded portion will expand as the press platens are backed away, leaving the central portion of the sheet of porous, felted structure and well adapted for insulating purposes. No precautions need be observed in opening the press platens if the temperature is first sufficiently reduced to avoid blowing out or disruptive action of steam but the press pressure should desirably be continued for a time after the steam supply to the press platens has been cut off in order to ensure suitable reduction of temperature before releasing the press.

Use of fiber in the form in which it comes from the gun without much or any refinement is advantageous by reason of its elastic nature and a good degree of interior porosity is obtained by expansion of the unwelded portion following pressure relief.

Pressures of from 200-700# per square inch, preferably from 400-500# per square inch, have been found to give very satisfactory results in producing surface portions of desirable hardness, density and strength, but wide variations in pressure, as from about 25-1200# per square inch may be resorted to, if desired, to obtain density and strength in the surface portions corresponding roughly

to the pressure used. When steam heated press platens are used the steam for heating the platens is preferably of a pressure over 50# per square inch, but considerably higher pressures and temperatures than this may be used so long as objectionable overheating and charring is avoided. With press platens heated by steam at about 100# per square inch and a pressure between the platens of about 400-500# per square inch a fiber sheet which is about 1½" thick as it comes from the squeezing rolls after being subjected to the heat and pressure for about 5-10 minutes and the press released upon the temperature being reduced as described has a thickness of approximately 1", of which the outer 1/8" or thereabouts on each surface is of hard, dense thoroughly consolidated and welded structure and the intervening portion approximately 3/4" in thickness is porous and of good insulating qualities. There can, of course, be a great deal of variation in respect of thicknesses and density of the product and the several portions thereof, according to requirements in connection with the use to which the board is to be put, and the time of heat cut-off and release of the press is gauged in accordance with the particular sort of product required, the pressure being continued for a less interval where the thickness, strength and density of the surface portions is relatively less important and for longer periods when surface portions of greater resisting qualities are required.

In order to obtain desirably good welded surface portions, any give or shrinkage taking place in the body of fiber should be followed up by the press platens, and the full pressure used should be maintained throughout the body of fibrous material, until the point of time is reached at which the heat is cut down followed by the pressure being intentionally released.

The drying is preferably completed, as, for example, in a drier or kiln after the sheets are removed from the press.

A board as above described, and having upper and lower welded portions and an intermediate porous insulating portion is produced when the body of felted fiber is pressed between heated upper and lower press platens. When, however, one of the press platens, as the lower one, is kept cold so that welding of the fibers does not take place in that part of the body of fiber adjacent to such cold platen and same expands after the press is released, a board product is obtained having but one surface portion of high denseness and a backing portion of the porous felted and non-welded fiber. The drying of the product can readily be completed in the press after the pressure is wholly or partly released, as by restoring the steam supply to the chambers in the press platens,

which supply had been cut off to reduce the temperature prior to releasing the press.

I claim:

1. Process of forming integral fiber products comprising adjacent portions which are respectively of high density and of high porosity, which comprises applying heat and pressure to a body of moist ligno-cellulose fiber until welding or coalescing of the fibers into permanent relation has extended therein to a material extent but not therethrough, cutting off the application of heat while still maintaining the pressure, and finally releasing the pressure.
- 15 2. Process of forming integral fiber products comprising adjacent portions which are respectively of high density and high porosity, which comprises applying heat and pressure to a moist body of wood or woody fiber, obtained by explosion from under a high pressure and containing practically all the original wood or woody material, until welding or coalescing of the fibers into permanent relation has extended therein to a material extent but not therethrough, cutting off the application of heat while still maintaining the pressure, and finally releasing the pressure.

In testimony whereof, I have signed my  
30 name hereto.

WILLIAM H. MASON.

35

40

45

50

55

60

65